# EUROPEAN PATENT SPECIFICATION

(11) **EP 3 392 367 B1**
(45) Date of publication and mention of the grant of the patent: **27.10.2021**
(21) Application number: 16876051.0
(22) Date of filing: 15.12.2016
(51) Int. Cl.: C22C 38/02, C22C 38/04, C22C 38/06, C22C 38/42, C22C 38/44, C22C 38/50, C22C 38/48, C22C 38/46, C22C 38/58, C22C 38/00, C21D 8/02, C21D 6/00, C21D 9/46

(54) **HIGH-STRENGTH STEEL MATERIAL HAVING EXCELLENT LOW-TEMPERATURE STRAIN AGING IMPACT PROPERTIES AND METHOD FOR MANUFACTURING SAME**
HOCHFESTES STAHLMATERIAL MIT HERVORRAGENDEN TIEFTEMPERATURZÄHIGKEITSBEANSPRUCHUNGSEIGENSCHAFTEN SOWIE VERFAHREN ZUR HERSTELLUNG DAVON
MATÉRIAU EN ACIER À HAUTE RÉSISTANCE AYANT D'EXCELLENTES PROPRIÉTÉS AU CHOC PAR VIEILLISSEMENT PAR CONTRAINTE À BASSE TEMPÉRATURE ET SON PROCÉDÉ DE FABRICATION

(30) Priority: 15.12.2015 KR 20150178977
(43) Date of publication of application: 24.10.2018
(73) Proprietor: POSCO, Pohang-si, Gyeongsangbuk-do 37859 (KR)
(72) Inventor: UM, Kyung-Keun, Pohang-si, Gyeongsangbuk-do 37877 (KR); KIM, Woo-Gyeom, Pohang-si, Gyeongsangbuk-do 37877 (KR); LEE, Hong-Ju, Pohang-si, Gyeongsangbuk-do 37877 (KR)
(74) Representative: Potter Clarkson
(86) International application number: PCT/KR2016/014734
(87) International publication number: WO 2017/105109

(56) References cited:
- EP-A1- 2 764 946
- EP-A1- 2 832 889
- WO-A1-2015/151468
- WO-A1-2017/105107
- JP-A- 2012 241 266
- JP-A- 2014 043 627
- KR-A- 20110 060 449
- KR-A- 20110 060 449
- KR-A- 20120 074 638
- KR-A- 20130 076 569
- KR-A- 20130 076 569
- KR-A- 20140 030 465
- KR-A- 20150 124 810
- KR-A- 20150 124 810

## Description

### [Technical Field]

The present disclosure relates to a steel material used as a material for pressure vessels, offshore structures and the like, and more particularly, to a high-strength steel material having excellent low-temperature strain aging impac8 t properties, and a method for manufacturing the same.

### [Background Art]

Recently, mining areas have moved to deep-sea areas or areas of extreme cold due to the exhaustion of energy resources, and thus, mining and storage facilities are becoming larger and more complicated. Steel materials used therein are required to have excellent low-temperature toughness for securing high strength and facility stability for reducing weight.

Meanwhile, since cold deformation often occurs in the course of manufacturing a steel material having strength and toughness as described above to form a steel pipe or other complicated structures, the steel material is required to significantly avoid a decrease in toughness due to strain aging by cold deformation.

The mechanism of decreased toughness due to strain aging is as follows: The toughness of a steel material measured by a Charpy impact test is explained by a correlation between yield strength and fracture strength at the test temperature; and when the yield strength of a steel material at the test temperature is higher than the fracture strength, the steel material undergoes brittle fracture without ductile fracture, so that an impact energy value is lowered, but when the yield strength is lower than the fracture strength, the steel material is deformed to be ductile, thereby absorbing impact energy during work hardening, and being changed to undergo brittle fracture when the yield strength reaches fracture strength. That is, as the difference between the yield strength and the fracture strength is larger, the amount of the steel material deformed to be ductile is increased, so that the impact energy to be absorbed is increased. Therefore, when subjecting the steel material to cold deformation for manufacturing to form a steel pipe or other complicated structure, the yield strength of the steel material is increased as deformation continues, and thus, the difference from the fracture strength becomes smaller, accompanied by decreased impact toughness.

Thus, in order to prevent decreased toughness by cold deformation, conventionally, a method of significantly decreasing the amount of carbon (C) or nitrogen (N) employed in the steel material, or adding an element (e.g., titanium (Ti) , vanadium (V), etc.) to precipitate those elements at a minimum amount or more, for suppressing strength increase by an aging phenomenon after deformation, a method of performing SR (stress relief) heat treatment after cold deformation to decrease dislocation and the like produced in the steel material, thereby lowering the yield strength increased by work hardening, a method of adding an element (e.g., nickel (Ni), etc.) to lower stacking fault energy to facilitate the movement of dislocations, for increasing ductility of the steel material at low temperature, and the like have been suggested, and applied.

However, as structures and the like are continuously becoming larger and more complicated, the cold deformation amount required for the steel material is increased, and also the temperature of a use environment is lowered to the level of arctic sea temperature. Thus, it is difficult to effectively prevent toughness decrease by strain aging of the steel material, with conventional methods.

(Non-patent document 1) Effect of Ti addition on strain aging of low-carbon steel wire rod (Ikuo Ochiai, Hiroshi Ohba, Iron and Steel, Volume 75 (1989), issue 4, p. 642-)

(Non-patent document 2) The effect of processing variables on the mechanical properties and strain ageing of high-strength low-alloy V and V-N steels (V. K. Heikkinen and J. D. Boyd, CANADIAN METALLURGICAL QUARTERLY Volume 15 Number 3 (1976), p. 219-)

KR 2013 0076569 A discloses a steel for use in manufacture of a pressure vessel and having good sulfide stress cracking resistance and low temperature toughness. The steel includes, by weight %, 0.03 to 0.18%C, 0.05 to 0.5% Si, 0.5 to 2% Mn, 0.005 to 0.1% A1, 0.15 to 0.5% Cu, 0.15 to 1% Ni, 0.01 to 0.05% Nb, 0.01 to 0.05% Ti, 0.05 to 0.3% Mo, 0.05 to 0.5% Cr, 0.001 to 0.003% Ca, 0.001 to 0.01% N, not more than 0.0015% S, not more than 0.012% P and the balance Fe and inevitable impurities. EP2764946 A1 discloses a welded steel pipe formed by cold-bending and welding a steel plate. The steel plate has a composition that seeks to maintain toughness of the weld heat-affected zone at relatively low temperatures. The composition of the steel plate is in weight % 0.03 to 0.08% C, 0.01 to 0.20% Si, 1.0 to 2.2% Mn, 0.015% or less P, 0.001 to 0.05% Al, 0.005 to 0.050% Nb, 0.005 to 0.030% Ti, 0.0020 to 0.0080% N and one or more selected from a group including Cu, Ni, Cr, Mo, V and B.
JP 2014 043627 A discloses a steel for use in a polyolefin-coated, low-temperature UOE steel pipe comprising, in weight %, 0.03 to 0.07% C, 0.05 to 0.50% Si, 1.4 to 2.2% Mn, 0.020% or less P, 0.003% or less S, 0.15 to 0.60% Cu, 0.15 to 0.80% Ni, 0.005 to 0.045% Nb, 0.005 to 0.030% Ti, 0.0070% or less N, 0.005 to 0.060% Al and the balance Fe and inevitable impurities.

### [Disclosure]

### [Technical Problem]

An aspect of the present disclosure is to provide a steel material which may not only secure high strength and high toughness, but may also significantly avoid a strength decrease due to cold deformation, thereby being appropriately applied as a material of pressure vessels, offshore structures and the like, and a method for manufacturing the same.

### [Technical Solution]

The invention is defined in the claims.

### [Advantageous Effects]

As set forth above, according to an exemplary embodiment in the present disclosure, a heat-treated steel material having excellent low-temperature stain aging impact properties, simultaneously with high strength may be provided, and the steel material may be appropriately applied as a material for pressure vessels, offshore structures and the like, following a trend of being larger and more complicated.

### [Description of Drawings]

FIG. 1 is a graph representing lower yield strength and tensile strength in a tensile curve of a steel material according to an aspect of the present disclosure.

### [Best Mode for Invention]

As the cold deformation amount for the steel material used as a material for pressure vessels, offshore structures and the like is continuously increased, the present inventors conducted an intensive study on the development of a steel material which may prevent a toughness decrease of the steel material by strain aging, while having high strength and high toughness, and as a result, confirmed that a steel material having a microstructure advantageous for securing the above-described physical properties from optimization of a steel component composition and manufacturing conditions may be provided, thereby completing the present disclosure.

In particular, the steel material of the present disclosure may effectively prevent a toughness decrease by strain aging by optimizing the contents of the elements having an influence on MA phase formation in the steel component composition to significantly decrease the MA phase (martensite-austenite composite phase).

Hereinafter, the present disclosure will be described in detail.

The high-strength steel material having excellent low-temperature strain aging impact properties according to an aspect of the present disclosure includes 0.04-0.14 wt% of carbon (C), 0.05-0.60 wt% of silicon (Si), 0.6-1.8 wt% of manganese (Mn), 0.005-0.06 wt% of soluble aluminum (sol. Al), 0.005-0.05 wt% of niobium (Nb), more than 0 wt% to 0.01 wt% of vanadium (V), 0.001-0.015 wt% of titanium (Ti), 0.01-0.4 wt% of copper (Cu), 0.01-0.6 wt% of nickel (Ni), 0.01-0.2 wt% of chromium (Cr), 0.001-0.3 wt% of molybdenum (Mo), 0.0002-0.0040 wt% of calcium (Ca), 0.001-0.006 wt% of nitrogen (N), more than 0 wt% to 0.02 wt% of phosphorus (P), and more than 0 wt% to 0. 003 wt% of sulfur (S) .

Hereinafter, the reason why the alloy components of the high-strength steel material provided by the present disclosure are controlled as described above will be described in detail. Herein, unless otherwise stated, the content of each component refers to wt%.

### C: 0.04-0.14%

Carbon (C), an element advantageous for securing strength of a steel is bonded to pearlite or niobium (Nb), nitrogen (N) and the like to exist as carbonitrides, and thus, is a main element for securing tensile strength. It is not preferable that the content of this C is less than 0.04%, since the tensile strength on a matrix may be lowered, and when the content is more than 0.14%, pearlite may be excessively produced, so that low-temperature strain aging impact properties may be deteriorated.

Therefore, the content of C is limited to 0.04-0.14%.

### Si: 0.05-0.60%

Silicon (Si), an element added for a deoxidation and desulfurization effect of a steel, and also for solid solution strengthening and is added at 0.05% or more for securing yield strength and tensile strength. However, it is not preferable that the content of silicon is more than 0 .60%, since weldability and low-temperature impact properties are lowered, and a steel surface is easily oxidized so that an oxide film may be severely formed.

Therefore, the content of Si is limited to 0.05-0.60%.

### Mn: 0.6-1.8%

Manganese (Mn) is added at 0.6% or more, since manganese has a large effect on strength increase by solid solution strengthening. However, when the content of Mn is excessive, segregation becomes severe in the center of a steel plate in the thickness direction, and at the same time formation of MnS, a nonmetallic inclusion, is encouraged, together with segregated S. The MnS inclusion produced in the center is stretched by rolling, and as a result, significantly deteriorates low-temperature toughness and lamella tear resistant properties, and thus, the content of Mn limited to 1.8% or less.

Therefore, the content of Mn is limited to 0.6-1.8%.

### Sol. Al: 0.005-0.06%

Soluble aluminum (sol. Al) is used as a strong deoxidizing agent in a steel manufacturing process together with Si, and 0.005% of sol. Al is added in deoxidation alone or in combination. However, when the content is more than 0.06%, the above-described effect is saturated, and the fraction of Al₂O₃ in the oxidative inclusion produced as a resultant product of deoxidation is increased more than necessary, and the size is larger. Thus, it is not easy to be removed during refining, resulting in significant reduction in low-temperature toughness, and thus, is not preferable.

Therefore, the content of Sol. Al is limited to 0.005-0.06%.

### Nb: 0.005-0.05%

Niobium (Nb) has a large effect of being solid-solubilized in austenite when reheating a slab, thereby increasing hardenability of austenite, and being precipitated as fine carbonitrides (Nb,Ti)(C,N) upon hot rolling, thereby suppressing recrystallization during rolling or cooling to allow a final microstructure to be finely formed. In addition, as the added amount of Nb is increased, the formation of bainite or MA is promoted to increase strength, however, it is not preferable that the content is more than 0.05%, since it is easy to form excessive MA, or a coarse precipitate in the center in the thickness direction, thereby deteriorating low-temperature toughness in the center of the steel.

Therefore, the content of Nb is limited to 0.005-0.05%, more advantageously 0.02% or more, still more advantageously 0.022% or more.

### V: 0.01% or less (exclusive of 0%)

Vanadium (V) is almost all solid-solubilized again when heating a slab, and thus, there is little effect of strength increase by precipitation or solid solubilization after rolling, normalizing heat treatment. In addition, V is an expensive element, and causes cost increase when adding it in a large amount, and thus, considering this, 0.01% or less of is added.

### Ti: 0.001-0.015%

Titanium (Ti) is present as a hexagonal precipitate mainly in the form of TiN at high temperature, or forms carbonitride (Nb,Ti) (C,N) precipitates with Nb and the like to suppress crystal grain growth in the welding heat-affected zone. For this, 0.001% or more of Ti is added. However, when the content is excessive and more than 0.015%, coarse TiN is formed in the center of the steel in the thickness direction, which serves as a fracture crack initiation point, thereby greatly reducing strain aging impact properties.

Therefore, the content of Ti is limited to 0.001-0.015%.

### Cu: 0.01-0.4%

Copper (Cu) has an effect of greatly improving strength by solid solubilization and precipitation, and not greatly affecting strain aging impact properties. However, when excessively added, it causes cracks on a steel surface, and is an expensive element, and thus, considering this, the content of Cu is limited 0.01-0.4%.

### Ni: 0.01-0.6%

Nickel (Ni) has little strength increase effect. However, it is effective in improving low-temperature strain aging impact properties, and in particular, when adding Cu, has an effect of suppressing a surface crack by selective oxidation which occurs upon reheating a slab. For this, 0.01% or more of Ni is added. However, considering the economic efficiency due to a high price, the content of Ni is limited to 0.6% or less.

### Cr: 0.01-0.2%

Chromium (Cr) has a small effect of increasing yield strength and tensile strength by solid solubilization. However, it slows down a cementite decomposition rate during heat treatment after welding or tempering, thereby preventing a drop in strength. For this, 0.01% or more of Cr is added. However, it is not preferable that the content is more than 0.2%, since the manufacturing cost rises, and also low-temperature toughness of the welding heat-affected zone is deteriorated.

### Mo: 0.001-0.3%

Molybdenum (Mo) has an effect of delaying transformation in the course of cooling after heat treatment, resulting in a large increase in strength, and also, being effective in preventing a drop in strength during heat treatment after welding or tempering like Cr, and preventing toughness decrease by grain boundary segregation of impurities such as P. For this, 0.001% or more of molybdenum is added. However, it is also economically disadvantageous to excessively add molybdenum, an expensive element, and thus, the content of Mo is limited to 0.3% or less.

### Ca: 0.0002-0.0040%

When calcium (Ca) is added after Al deoxidation, Ca is bonded to S which exists as MnS to inhibit production of MnS, simultaneously with formation of globular-shaped CaS, thereby having an effect of suppressing cracks in the center of the steel material. Therefore, in order to sufficiently transform S, added in the present disclosure, into CaS, 0.0002% or more is added.

However, when the content is more than 0.0040%, remaining Ca after forming CaS is bonded to O to produce a coarse oxidative inclusion, that becomes stretched and fractured in rolling to serve as a crack initiation point.

Therefore, the content of Ca is limited to 0.0002-0.0040%.

### N: 0.001-0.006%

Nitrogen (N) has an effect of being bonded to added Nb, Ti, Al, etc. to form a precipitate, thereby refining the crystal grains of the steel to improve the strength and toughness of a base metal. However, when the content is excessive, precipitates are formed, and remaining N exists in an atom state to cause aging after cold deformation. Thus, nitrogen is known as a representative element to decrease low-temperature toughness. In addition, when manufacturing a slab by continuous casting, surface cracks are promoted by embrittlement at high temperature.

Therefore, considering this, the content of N is limited to 0.001-0.006%.

### P: 0.02% or less (exclusive of 0%)

Phosphorus (P) has an effect of increasing strength when added. However, in the heat-treated steel of the present disclosure, it is an element which significantly impairs low-temperature toughness by grain boundary segregation, as compared with the effect of increasing strength, and thus it is preferable to keep the content of P as low as possible. However, since a significant cost is required to excessively remove P in a steel manufacturing process, the content of P is limited to the range not affecting the physical properties, i.e., 0.02% or less.

### S: 0.003% or less (exclusive of 0%)

Sulfur (S) is a representative factor bonded to Mn to produce a MnS inclusion in the center of the steel plate in the thickness direction, thereby deteriorating low-temperature toughness. Therefore, it is preferable to keep the content of S as low as possible for securing the low-temperature strain aging impact properties. However, since a significant cost is required to excessively remove this S, the content of S is limited to the range not affecting the physical properties, i.e., 0.003% or less.

The remaining component of the steel material is iron (Fe) . However, since in the common steel manufacturing process, unintended impurities may be inevitably incorporated from raw materials or the surrounding environment, they may not be excluded. Since these impurities are known to any person skilled in the common steel manufacturing process, the entire contents thereof are not particularly mentioned in the present specification.

The high-strength steel material of the present disclosure satisfying the alloy component composition as described above consists of a mixed structure of ferrite, pearlite, bainite and a MA (martensite-austenite) composite phase.

In the structure, ferrite is the most important since it allows the ductile deformation of the steel material, and it is included as a main phase, while finely controlling its average crystal grain size to 15 µm or less. As such, by refining ferrite crystal grains, a grain boundary may be increased to suppress crack propagation, basic toughness of a steel material may be improved, and also strength increase by an effect of lowering a work hardening rate during cold deformation may be significantly reduced, thereby improving strain aging impact properties simultaneously.

Hard phases including the pearlite, bainite, MA other than the ferrite is advantageous for securing high strength by increasing the tensile strength of a steel material. However, such phases serve as fracture initiation points or propagation paths due to high hardness, thereby deteriorating the strain aging impact properties. Therefore, the fraction is controlled, and the sum of fractions of the hard phases is more than 0% and is limited to 18% or less.

In particular, since the MA phase has the highest strength, and is transformed from martensite having strong brittleness by deformation, it is a phase which deteriorates the low-temperature toughness most significantly. Therefore, the fraction of the MA phase is more than 0% and is limited to 3.5% or less, and more preferably to 1.0-3.5%.

Meanwhile, the high-strength steel material of the present disclosure having the microstructure as described above includes carbonitrides produced by Nb, Ti, Al, etc., among the added elements, and the carbonitrides play an important role in inhibiting crystal grain growth in the course of rolling, cooling and heat treatment to allow the grains to be fine. In order to significantly increase the effect, the steel material includes 0.01% or more, and preferably 0.01-0.06% of the carbonitrides having an average size of 300 nm or less by weight ratio.

Hereinafter, a method for manufacturing a high-strength steel material having excellent low-temperature strain aging impact properties, another aspect of the present disclosure will be described in detail.

A steel slab satisfying the above-described alloy component alloy is manufactured, and then in order to obtain a steel material satisfying microstructure, carbide conditions and the like aimed at in the present disclosure, hot rolling (controlled rolling), cooling and normalizing heat treatment are performed.

Prior to this, the manufactured steel slab is subjected to a reheating process.

The reheating temperature is controlled to 1080-1250°C, and when the reheating temperature is less than 1080 °C, re-solid solubilization of carbides produced in the slab during continuous casting is difficult. Therefore, it is preferable to perform reheating to at least a temperature at which 50% or more of added Nb may be solid-solubilized again. However, when the temperature is more than 1250°C, the size of austenite crystal grains is unduly large, so that the mechanical physical properties such as strength and toughness of the finally manufactured steel material are greatly deteriorated.

Therefore, the reheating temperature is limited to 1080-1250°C.

Manufacture of the hot-rolled steel plate includes finish rolling of the reheated steel slab as described above. Herein, the finish rolling process is controlled rolling, and the rolling end temperature is controlled to be 780°C or more.

When rolling is performed by a common rolling process, the rolling end temperature is about 820-1000°C. However, when this is lowered to less than 780°C, the quenching property is lowered in the region in which Mn and the like are not segregated during rolling, thereby producing ferrite during rolling, and as the ferrite is produced as such, solid-solubilized C and the like are segregated into a remaining austenite region and concentrated. Accordingly, the region in which C and the like are concentrated during cooling after rolling is transformed into bainite, martensite or a MA phase, thereby producing a strong layered structure formed of ferrite and a hardened structure. The hardened structure of the layer in which C and the like are concentrated has high hardness and also a greatly increased fraction of the MA phase. Since low-temperature toughness is decreased by an increase of hardened structure and arrangement of a layered structure, the rolled end temperature is controlled to be 780°C or more.

The hot-rolled steel plate obtained by controlled rolling according to the above is cooled by air cooling or water cooling, and then is subject to normalizing heat treatment in a constant temperature range, thereby manufacturing a steel material having the desired physical properties.

The normalizing heat treatment is performed by maintaining a temperature range of 850-960°C for a certain period of time, and then cooling in the air. When the normalizing heat treatment temperature is less than 850°C, the re-solidification solubilization of cementite and a MA phase in pearlite and bainite is not readily able to decrease the solid-solubilized C, so that it is difficult to secure strength, and also, a finally remaining hardened phase remains coarse, thereby significantly impairing strain aging impact properties. However, when the temperature is more than 960°C, crystal grain growth occurs to deteriorate the strain aging impact properties.

The normalizing heat treatment temperature range is maintained for {(1.3×t)+(10-60)} minutes (wherein 't' denotes a steel material thickness (mm)). When the maintaining time is shorter than that, the uniformity of the structure is difficult to achieve; and when the time is longer than that, productivity is deteriorated.

The high-strength steel material obtained according to the above has excellent strength and toughness, and also may effectively prevent toughness decrease by strain aging upon cold deformation. In particular, a yield ratio (YS (lower yield strength) /TS (tensile strength)) after heat treatment of 0.65-0.80 may be secured.

### [Mode for Invention]

Hereinafter, the present disclosure will be specifically described through the following Examples. However, it should be noted that the following Examples are only for describing the present disclosure in detail by illustration, and not intended to limit the right scope of the present disclosure. The reason is that the right scope of the present disclosure is determined by the matters described in the claims and reasonably inferred therefrom.

### (Examples)

The steel slabs having the component composition shown in the following Table 1 were subjected to reheating, hot rolling and normalizing heat treatment under the conditions shown in the following Table 2, thereby manufacturing hot-rolled steel plates having a final thickness of 6 mm or more.

The microstructure fraction, size and carbonitride fraction of each of the manufactured hot-rolled steel plates were measured. In addition, a Charpy impact transition temperature was measured in the state of being aged at 250°C for 1 hour after 5% stretching of a cold deformation amount, which may represent strength (tensile strength and lower yield strength) and strain aging impact properties of each hot-rolled steel plate, and represented in the following Table 3.

For the microstructure of each hot-rolled steel plate, the steel plate section was polished with a mirror surface, and etched with Nital or Lepera as desired, thereby measuring an image for a certain area of a specimen at 100-500X magnification with an optical or scanning electron microscope, and then the fraction of each image was measured from the measured images using an image analyzer. In order to obtain a statistically significant value, the measurement was repeated for the same specimen but at the changed position, and the average value was calculated.

The fraction of the fine carbonitrides having an average size of 300 nm or less was measured by an extraction residue method.

As tensile property values, lower yield strength, tensile strength and a yield ratio (lower yield strength/tensile strength) were measured, respectively from a nominal strain-nominal stress curve obtained by a common tensile test, and a strain aging impact property value was measured by adding 0%, 5% and 8% in advance as a tensile strain, aging a stretched specimen at 250°C for 1 hour, and then performing a Charpy V-notch impact test.

(In the above Table 3, 'F fraction' refers to a ferrite fraction, and 'F size' refers to an average size of ferrite crystal grains.

In addition, the represented hardened phase fraction (%) includes the carbonitride fraction (%).)

As shown in the above Tables 1 to 3, the hot-rolled steel plate satisfying all of the component composition and manufacturing conditions of the present disclosure has high strength, and also secures excellent low-temperature toughness even after cold deformation, thereby being appropriately used in pressure vessels, offshore structures and the like, following a trend of being larger and more complicated.

In Comparative Examples 1 to 5 in which the manufacturing conditions satisfied the present disclosure, but the steel component composition did not satisfy the present disclosure, low strength or deteriorated low-temperature toughness were confirmed.

Among them, in Comparative Example 1 in which the content of C was not sufficient, the ferrite crystal grains were coarse following rolling and heat treating, so that sufficient strength was not secured.

In Comparative Example 2 in which the content of C was excessive, a hardened phase fraction was more than 18%, and the fraction of MA phase was greatly increased, thereby lowering the yield ratio, resulting in a high impact transition temperature after 5% cold deformation.

In Comparative Example 3 in which the content of Ti is excessive, Ti which was excessively added as compared with added N was produced as a coarse TiN precipitate, and when impacted after 5% cold deformation, served as an initiation point of cracks, resulting in a higher impact transition temperature.

In Comparative Example 4 in which the content of Nb was insufficient, due to phase transformation delay by Nb re-solid solubilization, a strengthening effect by crystal grain refining and precipitation producing was not exhibited to deteriorate strength.

In Comparative Example 5 in which the content of Cu was excessive, this Cu raises the solid solubilization of C in austenite when cooling after normalizing heat treatment, thereby increasing a MA phase fraction after final transformation, thereby lowering the yield ratio, and raising the impact transition temperature after 5% cold deformation.

## Claims

1. A high-strength steel material having excellent low-temperature strain aging impact properties, the steel material comprising: 0.04-0.14 wt% of carbon (C), 0.05-0.60 wt% of silicon (Si), 0.6-1.8 wt% of manganese (Mn), 0.005-0.06 wt% of soluble aluminum (sol. Al), 0.005-0.05 wt% of niobium (Nb), more than 0 wt% to 0.01 wt% of vanadium (V), 0.001-0.015 wt% of titanium (Ti), 0.01-0.4 wt% of copper (Cu), 0.01-0.6 wt% of nickel (Ni), 0.01-0.2 wt% of chromium (Cr), 0. 001-0. 3 wt% of molybdenum (Mo), 0. 0002-0 . 0040 wt% of calcium (Ca), 0.001-0.006 wt% of nitrogen (N), more than 0 wt% to 0.02 wt% of phosphorus (P), and more than 0 wt% to 0. 003 wt% of sulfur (S), with a balance of Fe and other inevitable impurities, and
consisting of a mixed structure of ferrite, pearlite, bainite and a martensite-austenite (MA) composite phase as a microstructure, wherein an area fraction of the MA phase is more than 0% to 3.5%, wherein a sum of area fractions of remaining phases, other than ferrite, is more than 0% to 18% or less,
wherein an average of ferrite crystal grain size is 15 µm or less, and
wherein the steel material comprises carbonitrides having an average size of 300 nm or less at 0.01% or more by weight ratio.

2. The high-strength steel material of claim 1, wherein the niobium (Nb) is comprised in an amount of 0.02-0.5%.

3. The high-strength steel material of claim 1, wherein a yield ratio defined as (lower yield strength) / (tensile strength) is 0.65-0.80.

4. A method for manufacturing a high-strength steel material of claim 1 having excellent low-temperature strain aging impact properties, the method comprising: reheating a steel slab including 0.04-0.14 wt% of carbon (C), 0.05-0.60 wt% of silicon (Si), 0.6-1.8 wt% of manganese (Mn), 0.005-0.06 wt% of soluble aluminum (sol. Al), 0. 005-0. 05 wt% of niobium (Nb), more than 0 wt% to 0.01 wt% of vanadium (V), 0.001-0.015 wt% of titanium (Ti), 0.01-0.4 wt% of copper (Cu), 0.01-0.6wt% of nickel (Ni), 0.01-0.2 wt% of chromium (Cr), 0.001-0.3 wt% of molybdenum (Mo), 0.0002-0.0040 wt% of calcium (Ca), 0.001-0.006 wt% of nitrogen (N), more than 0 wt% to 0.02 wt% of phosphorus (P), and more than 0 wt% to 0. 003 wt% of sulfur (S), with a balance of Fe and other inevitable impurities in a temperature range of 1080-1250°C;
controlled rolling the reheated slab so that a rolling end temperature is 780°C or more, whereby the slab is manufactured into a hot-rolled steel plate;
cooling the hot-rolled steel plate by air cooling or water cooling; and
after the cooling, subjecting the hot-rolled steel plate to normalizing heat treatment in a temperature range of 850-960°C, wherein the normalizing heat treatment is performed for (1.3t)+(10-60) minutes where 't' refers to a steel material thickness in mm.

5. The method of claim 4, wherein the steel slab includes 0.02-0.05% of niobium (Nb).

6. The method of claim 4, wherein the reheated slab is formed of 50% or more of Nb being solid-solubilized again.

## Patentansprüche

1. Hochfestes Stahlmaterial, das ausgezeichnete Niedertemperaturreckalterungsschlageigenschaften aufweist, wobei das Stahlmaterial Folgendes umfasst: 0,04-0,14 Gew.-% Kohlenstoff (C), 0,05-0,60 Gew.-% Silizium (Si), 0,6-1,8 Gew.-% Mangan (Mn), 0,005-0,06 Gew.-% lösliches Aluminium (Iösl. Al), 0,005-0,05 Gew.-% Niob (Nb), mehr als 0 Gew.-% bis 0,01 Gew.-% Vanadium (V), 0,001-0,015 Gew.-% Titan (Ti), 0,01-0,4 Gew.-% Kupfer (Cu), 0,01-0,6 Gew.-% Nickel (Ni), 0,01-0,2 Gew.-% Chrom (Cr), 0,001-0,3 Gew.-% Molybdän (Mo), 0,0002-0,0040 Gew.-% Kalzium (Ca), 0,001-0,006 Gew.-% Stickstoff (N), mehr als 0 Gew.-% bis 0,02 Gew.-% Phosphor (P) und mehr als 0 Gew.-% bis 0,003 Gew.-% Schwefel (S), mit einem Rest von Fe und anderen unvermeidlichen Verunreinigungen, und
aus Folgendem besteht
einer Mischstruktur aus Ferrit, Perlit, Bainit und einer Martensit-Austenit(MA)-Verbundwerkstoffphase als einer Mikrostruktur, wobei ein Flächenanteil der MA-Phase mehr als 0 % bis 3,5 % beträgt, wobei eine Summe der Flächenanteile verbleibender Phasen, außer Ferrit, mehr als 0 % bis 18 % oder weniger beträgt,
wobei eine durchschnittliche Ferritkristallkorngröße 15 µm oder weniger beträgt und
wobei das Stahlmaterial Karbonitride umfasst, die eine durchschnittliche Größe von 300 nm oder weniger bei einem Gew.-%-Verhältnis von 0,01 % oder mehr aufweisen.

2. Hochfestes Stahlmaterial nach Anspruch 1, wobei das Niob (Nb) in einer Menge von 0,02-0,5 % umfasst ist.

3. Hochfestes Stahlmaterial nach Anspruch 1, wobei ein Streckgrenzenverhältnis, das als (niedrigere Streckgrenze)/(Zugfestigkeit) definiert ist, 0,65-0,80 beträgt.

4. Verfahren zum Fertigen eines hochfesten Stahlmaterials nach Anspruch 1, das ausgezeichnete Niedertemperaturreckalterungsschlageigenschaften aufweist, wobei das Verfahren Folgendes umfasst: Anlassen einer Stahlbramme, die Folgendes beinhaltet: 0,04-0,14 Gew.-% Kohlenstoff (C), 0,05-0,60 Gew.-% Silizium (Si), 0,6-1,8 Gew.-% Mangan (Mn), 0,005-0,06 Gew.-% lösliches Aluminium (lösl. AI), 0,005-0,05 Gew.-% Niob (Nb), mehr als 0 Gew.-% bis 0,01 Gew.-% Vanadium (V), 0,001-0,015 Gew.-% Titan (Ti), 0,01-0,4 Gew.-% Kupfer (Cu), 0,01-0,6 Gew.-% Nickel (Ni), 0,01-0,2 Gew.-% Chrom (Cr), 0,001-0,3 Gew.-% Molybdän (Mo), 0,0002-0,0040 Gew.-% Kalzium (Ca), 0,001-0,006 Gew.-% Stickstoff (N), mehr als 0 Gew.-% bis 0,02 Gew.-% Phosphor (P) und mehr als 0 Gew.-% bis 0,003 Gew.-% Schwefel (S), mit einem Rest von Fe und anderen unvermeidlichen Verunreinigungen in einem Temperaturbereich von 1080-1250 °C;
gesteuertes Walzen der angelassenen Bramme, sodass eine Walzendtemperatur 780 °C oder mehr beträgt, wodurch die Bramme zu einem warmgewalzten Stahlblech gefertigt wird;
Abkühlen des warmgewalzten Stahlblechs durch Luftkühlen oder Wasserkühlen; und
nach dem Abkühlen, Unterziehen des warmgewalzten Stahlblechs unter eine normalisierende Wärmebehandlung in einem Temperaturbereich von 850-960 °C, wobei die normalisierende Wärmebehandlung für (1,3 t) + (10―60) Minuten durchgeführt wird, wobei "t" sich auf eine Stahlmaterialdicke in mm bezieht.

5. Verfahren nach Anspruch 4, wobei die Stahlbramme 0,02-0,05 % Niob (Nb) beinhaltet.

6. Verfahren nach Anspruch 4, wobei die angelassene Bramme aus 50 % oder mehr Nb ausgebildet wird, das wieder in einem Festlösungszustand ist.

## Revendications

1. Matériau en acier à haute résistance doté d'excellentes propriétés d'impact de vieillissement après déformation à basse température, le matériau en acier comprenant : 0,04 à 0,14 % en poids de carbone (C), 0,05 à 0,60 % en poids de silicium (Si), 0,6 à 1,8 % en poids de manganèse (Mn), 0,005 à 0,06 % en poids d'aluminium soluble (sol. Al), 0,005 à 0,05 % en poids de niobium (Nb), plus de 0 % en poids à 0,01 % en poids de vanadium (V), 0,001 à 0,015 % en poids de titane (Ti), 0,01 à 0,4 % en poids de cuivre (Cu), 0,01 à 0,6% en poids de nickel (Ni), 0,01 à 0,2 % en poids de chrome (Cr), 0,001 à 0,3 % en poids de molybdène (Mo), 0,0002 à 0,0040 % en poids de calcium (Ca), 0,001 à 0,006 % en poids d'azote (N), plus de 0 % en poids à 0,02 % en poids de phosphore (P) et plus de 0 % en poids à 0,003 % en poids de soufre (S), avec un reste de Fe et d'autres impuretés inévitables, et constitué d'une structure mixte de ferrite, de perlite, de bainite et d'une phase composite de martensite-austénite (MA) en tant que microstructure, dans lequel une fraction de surface de la phase MA est comprise entre plus de 0 % et 3,5 %, une somme des fractions de surface des phases restantes, autre que le ferrite, est supérieure ou inférieure à 0 % à 18 %,
dans lequel une moyenne de la taille de grain de cristal de ferrite est de 15 µm ou moins, et
dans lequel le matériau en acier comprend des carbonitrures ayant une taille moyenne de 300 nm ou moins à un rapport en poids de 0,01 % ou plus.

2. Matériau en acier à haute résistance selon la revendication 1, dans lequel le niobium (Nb) est compris en une quantité de 0,02 à 0,5 %.

3. Matériau en acier à haute résistance selon la revendication 1, dans lequel un taux d'extraction défini comme (résistance d'extraction inférieure)/(résistance à la traction) est de 0,65 à 0,80.

4. Procédé de fabrication d'un matériau en acier à haute résistance selon la revendication 1, ayant d'excellentes propriétés d'impact de vieillissement après déformation à basse température, le procédé comprenant : le réchauffage d'une brame d'acier comportant 0,04 à 0,14 % en poids de carbone (C), 0,05 à 0,60 % en poids de silicium (Si), 0,6 à 1,8 % en poids de manganèse (Mn), 0,005 à 0,06 % en poids d'aluminium soluble (sol. Al), 0,005 à 0,05 % en poids de niobium (Nb), plus de 0 % en poids à 0,01 % en poids de vanadium (V), 0,001 à 0,015 % en poids de titane (Ti), 0,01 à 0,4 % en poids de cuivre (Cu), 0,01 à 0,6 % en poids de nickel (Ni), 0,01 à 0,2 % en poids de chrome (Cr), 0,001 à 0,3 % en poids de molybdène (Mo), 0,0002 à 0,0040 % en poids de calcium (Ca), 0,001 à 0,006 % en poids d'azote (N), plus de 0 % en poids à 0,02 % en poids de phosphore (P) et plus de 0 % en poids à 0,003 % en poids de soufre (S), avec un reste de Fe et d'autres impuretés inévitables dans une plage de température de 1 080 à 1 250 °C ;
le laminage contrôlé de la brame réchauffée de telle sorte qu'une température finale de laminage soit de 780 °C ou plus, par lequel la brame est transformée en une tôle d'acier laminée à chaud ;
le refroidissement de la tôle d'acier laminée à chaud par refroidissement à l'air ou à l'eau ; et
après le refroidissement, la soumission de la tôle d'acier laminée à chaud à un traitement thermique de normalisation dans une plage de température de 850 à 960 °C, le traitement thermique de normalisation étant effectué pendant (1,3 t) + (10 à 60) minutes où « t » se réfère à une épaisseur de matériau en acier en mm.

5. Procédé selon la revendication 4, dans lequel la brame d'acier comprend 0,02 à 0,05 % de niobium (Nb).

6. Procédé selon la revendication 4, dans lequel la brame réchauffée est formée de 50 % ou plus de Nb étant à nouveau solubilisé sous forme solide.
